

# UNITED STATES PATENT OFFICE.

FREDERICK COATES, OF CINCINNATI, OHIO, ASSIGNOR TO FEDERAL PRODUCTS COMPANY, OF CINCINNATI, OHIO, A CORPORATION OF OHIO.

## PAPER-COATING COMPOSITION.

1,414,256.

Specification of Letters Patent. Patented Apr. 25, 1922.

No Drawing.

Application filed April 27, 1921. Serial No. 464,835.

To all whom it may concern:

Be it known that FREDERICK COATES, a citizen of the United States, residing at Cincinnati, in the county of Hamilton and State 5 of Ohio, has invented certain new and useful Improvements in Paper-Coating Composition, of which the following is a specification.

This invention relates to the coating of paper and especially to paper oil-proofing.

10 More particularly the invention relates to a paper oil-proofing composition and the method of manufacturing the same.

It is a well understood fact that paper cans or containers which are used for the packing 15 or storing of certain classes of substances such as butter, lard and other greases, as well as for storing and packing various other commodities, must be rendered proof against action by oil or the like.

20 One important object of the present invention is to provide an improved composition for oil-proofing paper.

A second important object of the invention 25 is to provide an improved composition for coating the interior or exterior of paper containers such as cans, or cartons.

A third important object of the invention is a provision of an improved composition for this purpose which dries very slowly, 30 does not sour or decompose readily and forms a superior preservative for the container.

A fourth important object of the invention is to provide an improved composition of this character which is elastic in its nature 35 so that it will not crack, or spall off from the container as do brittle compositions.

With the above and other objects in view as will be hereinafter understood the invention consists in general of a certain novel 40 composition of matter and an improved manner of manufacturing the same.

In the preparation of this composition there is taken one part of gelatin and two parts of water. The gelatin is immersed in 45 the water, both being at the ordinary atmospheric temperature and the gelatin and water are then allowed to stand for two hours, remaining during this period at substantially the same temperature as the atmosphere.

50 At the end of the two hours heat is applied and the temperature is raised to 120° Fahrenheit. When this temperature has been

reached there is added to the mixture one part of glucose and one-half part of glycerine. This mixture is kept at 120°. In the 55 meantime a second mixture is made which consists of two parts of water, one and one-half parts of glucose, one-half part of glycerine and one part of acetone. This mixture is made at the normal atmospheric tempera- 60 ture.

The two mixtures having been prepared they are slowly merged. The resultant mixture will have a temperature of about 110° in which condition it is applied to the 65 surface of the container in any desired manner. It is found that by making the two mixtures separately and then merging the two the resultant compound dries very slowly and remains sweet, and having practically no 70 tendency to sour. It is also found that this composition, formed in this manner, makes a highly efficient preservative which possesses such an amount of elasticity, as to render it peculiarly adapted for coating 75 paper cans and other containers.

Having thus described the invention, what is claimed as new, is:—

1. The process of forming a paper oil-proofing composition which consists in 80 merging two mixtures, one of said mixtures containing water, gelatin, glucose and glycerine and the other of said mixtures containing water, glucose, glycerine and acetone.

2. The process of forming a paper oil-proofing composition which consists in merging two mixtures, one of said mixtures containing two parts of water, one part of gelatin, one part of glucose and one-half part of glycerine, the other of said mixtures containing two parts water, one and one-half parts glucose, one-half part of glycerine, and one part of acetone.

3. The process of forming a paper oil-proofing composition which consists in merging two mixtures, one of said mixtures being formed by mixing two parts of water with one part of gelatin at normal atmospheric temperature and allowing the same to stand for two hours, raising the temperature of 100 the water and gelatin to 120°, adding one part of glucose and one-half part of glycerine thereto and maintaining the mixture at 120°, the other of said mixtures being

formed by mixing at normal atmospheric temperature two parts of water, one and one-half parts glucose, one-half part of glycerine and one part of acetone.

5 4. A paper oil-proofing composition comprising water, gelatin, glucose, glycerine, and acetone.

5. A paper oil-proofing composition consisting of four parts of water, one part of gelatin, two and one-half parts of glucose, one part of glycerine, and one part of acetone. 10

In testimony whereof I affix my signature.

FREDERICK COATES.